# EUROPEAN PATENT SPECIFICATION

(11) **EP 3 539 688 B1**
(45) Date of publication and mention of the grant of the patent: **06.07.2022**
(21) Application number: 19158971.2
(22) Date of filing: 23.02.2019
(51) Int. Cl.: B22C 9/28, B22D 18/04, B22C 9/06

(54) **LOW-PRESSURE CASTING MULTI-SPRUE PROCESS AND DEVICE FOR ALUMINUM ALLOY WHEEL**
NIEDERDRUCKGIESSVERFAHREN UND VORRICHTUNG MIT MEHREREN ANGÜSSEN FÜR ALUMINIUMLEGIERUNGSRAD
PROCÉDÉ MULTIDESCENTE DE COULÉE BASSE PRESSION ET DISPOSITIF DE ROUE EN ALLIAGE D'ALUMINIUM

(30) Priority: 13.03.2018 CN 201810204230
(43) Date of publication of application: 18.09.2019
(73) Proprietor: Citic Dicastal Co., Ltd., 066011 Quinhuangdao, Heibei (CN)
(72) Inventor: Du, Dexi, Qinhuangdao, Heibei 066011 (CN); Li, Changhai, Qinhuangdao, Heibei 066011 (CN)
(74) Representative: Gong, Jinping

(56) References cited:
- CN-A- 104 785 732
- CN-U- 207 723 471
- GB-A- 2 253 171
- JP-A- H07 155 928
- JP-A- 2000 237 862

## Description

### Field of the Invention

The present invention provides a low-pressure casting multi-sprue process and device for an aluminum alloy wheel.

### Background of the Invention

At present, the conventional low-pressure casting of aluminum alloy wheels mostly adopts a center bottom injection process. Molten aluminum enters a mold cavity through a center sprue, flows across the spokes of a wheel, and then turns to fill the rim vertically, until the filling is completed. In the process of crystallization and solidification, the rim is at a distal end far away from the center sprue and is solidified first. Therefore, it is necessary to preferentially feed the rim by the spokes to delay the crystallization and solidification time of the spokes, which affects the mechanical properties of the aluminum alloy wheel materials. Particularly, the elongation of the spokes is generally low, which directly affects the overall quality of the wheel.

JP 2000 237862 A relates to relates to low-pressure casting method and mold used in the casting of a vehicle wheel, such as a light alloy.

JP H07 155928 A relates to a mold structure of the vehicle wheel integrally forming the disk portion and a rim portion by the pressure casting of injecting molten metal by using the gas pressure.

CN 104 785 732 A discloses a wheel hub casting mold which comprises a mold base, wherein a fixed mold and a movable mold are fixed on the mold base.

### Summary of the Invention

The object of the present invention is to overcome the defects of the prior art, improve the quality of an aluminum alloy wheel by providing a low-pressure casting multi-sprue process for an aluminum alloy wheel, as specified in any one of claims 1-3, which focus on improving the elongation of spokes of the wheel and improving the casting production efficiency at the same time.

The technical solution adopted by the invention is: a low-pressure casting multi-sprue process for an aluminum alloy wheel adopts a multi-sprue casting method, and a plurality of sprues are arranged at the end of the inner rim of a wheel, so that molten aluminum enters the inner rim first, then enters from a center sprue after a mold cavity at the rim is full of the molten aluminum, and is pressurized and cooled after the mold cavity is full of the molten aluminum.

During cooling, starting from the outer rim of the wheel filled with the molten aluminum last, side mold ring water coolers are started, and the water coolers are close to the thick portions of the junctions of the spokes of the outer rim and the rim. Top mold coolers are also ring water coolers, the water coolers are located on a top mold above the spokes, and a center water cooler is adopted in the center of the top mold to cool the center sprue.

By controlling the cooling time and the flow rate, the molten aluminum in the cavity crystallizes in sequence with the cooling of the mold. The crystallization progresses from the outer rim to the rim and the spokes at the same time until the inner rim and the center of the wheel are finally solidified, completing the entire casting process.

In the low-pressure casting process, the front sides of the spokes and the outer rim of the wheel casting are upward, and the rim and the inner rim are at the lower part.

The plurality of sprues at the inner rim are arranged directly below the inner rim, the sprues are circular, and the number of the sprues varies according to the size of the wheel and is at least 8.

The center sprue is arranged directly below the center of the wheel, and is circular.

The side mold ring water cooler and the top mold ring water cooler are 15-40 mm away from the surface of the casting, and the flow rate of the cooling water is 150-400 L/hr.

A low-pressure casting device for an aluminum alloy wheel includes a cooling forming mold system and a pressure casting system, the casting device includes a multi-sprue mold, the lower part of the mold communicates with a sprue basin and is fixedly mounted on a machine bed plate, a low-pressure holding furnace is below the machine bed plate, and the molten aluminum in the furnace is connected to the central inlet of the sprue basin via a riser tube.

Atop mold and a side mold of the low-pressure casting mold are connected with a hydraulic control system of a machine, and the top mold is provided with an ejection mechanism for de-molding the casting.

A plurality of sprues are arranged at the junction of the sprue basin and the mold, a sprue bushing made of ceramic is arranged at each sprue, and the molten aluminum is finally crystallized and solidified at the sprue in the pressure feeding phase after filling of the molten aluminum.

Since a plurality of small sprues are arranged below the inner rim of the wheel and a center sprue is arranged in the center of the wheel at the same time, the filling time of the molten aluminum is shortened by half and the filling production efficiency is improved; the outer rim begins to solidify in the cooling process, and the spokes and the rim are simultaneously solidified in sequence, so that the crystallization and solidification time of the casting at the rim and the spokes is greatly shortened, the compactness of the internal structure of the casting is improved, the mechanical properties of the materials are good, and particularly, the elongation of the spokes is greatly improved; at the same time, the entire casting device is simple; and a sprue basin is added on the basis of ordinary low-pressure center casting, so that the whole process is simple and easy to operate.

### Brief Description of the Drawing

The present invention will be further illustrated below in conjunction with the drawing and embodiments.

Fig. 1 is a casting schematic diagram of a low-pressure multi-sprue process according to the present invention.

### Detailed Description of the Embodiments

In Fig. 1, a low-pressure casting multi-sprue process device for an aluminum alloy wheel according to the present invention mainly includes a mold cooling system and a pressure casting system. The casting mold includes a bottom mold (2), atop mold (4), a side mold (3) and a casting ejection rod (8). The entire mold is placed on a sprue basin (1). The mold cavity communicates with the sprue basin through a plurality of sprue bushings (11). The sprue basin is assembled on a machine bed plate (12) of a low-pressure casting main machine, a riser tube (13) is mounted therebetween to communicate with molten aluminum in a holding furnace (14), and the molten aluminum enters the sprue basin under the action of pressure through the riser tube, and then enters the mold cavity through the sprue bushings.

The mold cooling system includes side mold ring water coolers (9) and (10), top mold ring water coolers (6) and (7) and a center sprue spreader water cooler (5). The side mold ring water coolers are quickly started after the mold is full of the molten aluminum, a casting begins to crystallize and solidify at the outer rim, and the top mold ring water coolers and the center water cooler are sequentially started until the casting is solidified in sequence.

## Claims

1. A low-pressure casting multi-sprue process for an aluminum alloy wheel, **characterized in that** the casting process adopts a multi-sprue casting method, and a plurality of sprues are arranged at the end of the inner rim of a wheel, so that molten aluminum enters the inner rim first, and then enters from a center sprue after a mold cavity at the rim is full of the molten aluminum, **characterized in that**
during cooling, starting from the outer rim of the wheel filled with the molten aluminum last, side mold ring water coolers are started, and the water coolers are close to the thick portions of the junctions of the spokes of the outer rim and the rim; top mold coolers are also ring water coolers, the water coolers are located on a top mold above the spokes, and a center water cooler is adopted in the center of the top mold to cool the center sprue, wherein by controlling the cooling time and the flow rate, the molten aluminum in the cavity crystallizes in sequence with the cooling of the mold, wherein the crystallization progresses from the outer rim to the rim and the spokes at the same time until the inner rim and the center of the wheel are finally solidified, completing the entire casting process, wherein the side mold ring water coolers and the top mold ring water coolers are 15-40 mm away from the surface of the casting, the flow rate of cooling water is 150-400 L/hr, and the side mold ring water coolers need to be started immediately after the mold cavity is full of the molten aluminum.

2. The low-pressure casting multi-sprue process for an aluminum alloy wheel according to claim 1, **characterized in that** in the low-pressure casting process, the front sides of the spokes and the outer rim of the wheel casting are upward, and the rim and the inner rim are at the lower part.

3. The low-pressure casting multi-sprue process for an aluminum alloy wheel according to claim 1, **characterized in that** a plurality of sprues are arranged directly below the inner rim, a center sprue is arranged in the center, and the sprues are circular.

## Patentansprüche

1. Niederdruck-Mehranguß-Gießverfahren für ein Aluminiumlegierungsrad, **dadurch gekennzeichnet, dass** das Gießverfahren ein Mehranguß-Gießverfahren anwendet und eine Vielzahl von Angüssen am Ende der inneren Felge eines Rades angeordnet sind, so dass geschmolzenes Aluminium zuerst in die innere Felge eintritt und dann von einem zentralen Anguß eintritt, nachdem ein Formhohlraum an der Felge mit geschmolzenem Aluminium gefüllt ist, **dadurch gekennzeichnet, dass**
während des Abkühlens, ausgehend von der äußeren Felge des zuletzt mit dem geschmolzenen Aluminium gefüllten Rades, seitliche Formring-Wasserkühler gestartet werden, und die Wasserkühler sich in der Nähe der dicken Abschnitte der Verbindungen der Speichen der äußeren Felge und der Felge befinden; wobei Oberformkühler auch Ringwasserkühler ist, die Wasserkühler sich auf einer Oberform über den Speichen befinden, und wobei ein Mittelwasserkühler in der Mitte der Oberform verwendet wird, um den zentralen Anguß zu kühlen, wobei durch Steuern der Kühlzeit und der Fließgeschwindigkeit das geschmolzene Aluminium in der Kavität nacheinander mit dem Abkühlen der Form kristallisiert wird, wobei die Kristallisation von der äußeren Felge zur Felge und den Speichen gleichzeitig fortschreitet, bis die innere Felge und die Radmitte schließlich erstarrt sind, wird der gesamte Gießprozesses abgeschlossen, wobei die seitlichen Formring-Wasserkühler und die oberen Formring-Wasserkühler 15-40 mm von der Oberfläche des Gussstücks entfernt sind, die Durchflussrate des Kühlwassers 150-400 L/h beträgt, und die Seitenformring-Wasserkühler sofort gestartet werden müssen, nachdem der Formhohlraum mit geschmolzenem Aluminium gefüllt ist.

2. Niederdruck-Mehranguß-Gießverfahren für ein Aluminiumlegierungsrad nach Anspruch 1, **dadurch gekennzeichnet, dass** im Niederdruckgussverfahren die Speichenstirnseiten und der äußere Felge des Radgusses nach oben gerichtet sind, und die Felge und die innere Felge sich im unteren Teil befinden.

3. Niederdruck-Mehranguß-Gießverfahren für ein Aluminiumlegierungsrad nach Anspruch 1, **dadurch gekennzeichnet, dass** mehrere Angüsse direkt unterhalb des inneren Felge angeordnet sind, ein zentraler Anguß in der Mitte angeordnet ist und die Angüsse kreisförmig sind.

## Revendications

1. Un procédé de coulage multi-coulée à basse pression pour une roue en alliage d'aluminium, **caractérisé en ce que** le procédé de coulage adopte un procédé de coulage multi-coulée, et une pluralité de coulée sont disposé à l'extrémité du rebord intérieure d'une roue, de sorte que la matière fondue l'aluminium pénètre d'abord dans le rebord intérieur, puis pénètre à partir d'une coulée centrale après qu'une cavité de moule au niveau du rebord est remplie d'aluminium fondu, **caractérisé en ce que**
lors du refroidissement, en partant du rebord extérieure de la roue remplie de l'aluminium en fusion en dernier, des refroidisseurs d'eau à anneau de moule latéral sont mis en marche, et les refroidisseurs d'eau sont proches des parties épaisses des jonctions des rayons du rebord extérieure et du rebord; les refroidisseurs de moule de haut sont également des refroidisseurs d'eau annulaires, les refroidisseurs d'eau sont situés sur un moule de haut au-dessus des rayons, et un refroidisseur d'eau central est adopté au centre du moule de haut pour refroidir la coulée centrale, dans lequel en contrôlant le temps de refroidissement et la vitesse d'écoulement, l'aluminium fondu dans la cavité cristallise en séquence avec le refroidissement du moule, dans lequel la cristallisation progressant du rebord extérieur vers le rebord et les rayons en même temps jusqu'à ce que le bord intérieur et le centre de la roue soient finalement solidifiés, complétant l'ensemble du processus de coulée, dans lequel les refroidisseurs d'eau de l'anneau de moule latéral et les refroidisseurs d'eau de l'anneau de moule de haut sont à 15-40 mm de la surface de coulage, le vitesse d'écoulement d'eau de refroidissement est de 150 à 400 L/hr, et le les refroidisseurs d'eau à anneau de moule latéral doivent être démarrés immédiatement après que la cavité du moule est pleine d'aluminium fondu.

2. Le procédé de coulage multi-coulée à basse pression pour une roue en alliage d'aluminium selon la revendication 1, **caractérisé en ce que** dans le procédé de coulage à basse pression, les côtes avant des rayons et le rebord extérieure de la roue coulée sont vers le haut, et le rebord et le rebord intérieur sont à la partie basse.

3. Le procédé de coulage multi-coulée à basse pression pour une roue en alliage d'aluminium selon la revendication 1, **caractérisé en ce qu'**une pluralité de coulée sont disposées directement sous le rebord intérieure, une coulée centrale est disposée au centre et les coulée sont circulaires.
